

## UNITED STATES PATENT OFFICE

MARINO GENTILE, OF CHICAGO, ILLINOIS, ASSIGNOR, BY DIRECT AND MESNE ASSIGNMENTS, OF ONE-HALF TO SAMUEL W. WEIS, ONE-FOURTH TO GEORGE PICK, AND ONE-TWENTIETH TO HERBERT P. SHERWOOD, ALL OF CHICAGO, ILLINOIS

## TRANSPARENT SHEET

No Drawing.

Application filed June 26, 1929. Serial No. 373,951.

This invention relates to transparent sheets, films or containers such as are extensively used for wrapping or containing food and other products in sanitary display packages, for providing windows in window envelopes, and for various other purposes and applications. The main object of the invention is to provide a sheet, film or container for such purposes as those above indicated that can be made at a very low cost, shall be highly transparent, shall possess the strength, durability, and general efficiency of more expensive articles employed for the same purposes, and sufficiently moisture and grease proof to be practical.

In carrying out my present invention I take a sheet of thin paper as the base, preferably a soft, absorbent tissue, and this sheet I treat with a solution of cellulose nitrate dissolved in a suitable solvent such as ethyl acetate or amyl acetate, sufficient in amount to yield a suitable flowing solution. To this cellulose nitrate solution is then added a non-hygroscopic material which causes the treating solution to penetrate the paper base, and also renders the product soft and pliable when dry. Materials which satisfactorily serve these purposes are castor oil and tri cresyl phosphate but other materials possessing similar functional characteristics may be employed.

The treating solution can be applied to the paper base in any suitable manner, as by dipping the base sheet in, or drawing it through a body of the treating solution, or by flowing the latter over, or brushing, spraying or printing it on, the base sheet. The solution thoroughly penetrates and impregnates the fibrous structure of the base, and the latter is then dried. The residual product is a tough, flexible sheet highly transparent rendering completely visible objects covered thereby, non-porous and impervious to dust, grease and moisture, and thus well adapted to serve the purpose of a sanitary wrapper or container especially for food products, pharmaceutical products, and the like, and low in cost of materials and manufacture.

While I have described the invention

chiefly as embodied in sheet form, I do not limit it to such form but include within the spirit and purview of the claim molded or otherwise fabricated forms serving as holders or receptacles.

55

I claim:

As a new article of manufacture, a thin, tough, flexible, highly transparent, grease and moisture proof sheet having a base of thin, soft, absorbent tissue paper impregnated with and having a coating consisting essentially of cellulose nitrate integrally united therewith, the said coating substantially increasing the transparency of the paper base.

65

MARINO GENTILE.

70

75

80

85

90

95

100